

## UNITED STATES PATENT OFFICE

1,983,271

## PURIFICATION OF SAND

Theodore Earle, Denver, Colo.

No Drawing. Application September 19, 1932,  
Serial No. 633,851. Renewed April 10, 1934

14 Claims. (Cl. 252—8)

My invention which I call my dry leaching process relates to a process which will remove small amounts of impurities such as iron oxide, alumina, manganese oxide, and the like from 5 glass-sand, crushed feldspar and lepidolite, or other granular material, so that the ores or material may be made into more desirable products.

The object of my process is to reduce the 10 amount of harmful ingredients in an ore or material such as the above and do this at a low cost both for chemicals, treatment, and equipment needed to handle the material.

In my former patent application, Serial Number 511,446, filed January 26, 1931, I used dilute acid and brought this to the concentrated form by heating and evaporating the excess water in the diluent and thereby leaving a film of hot, concentrated acid around each sand grain to 20 act on the impurities.

The dissolved impurities are then washed free of the material. This process is even now in 25 successful commercial operation but, from the cost standpoint, it has two drawbacks. First—the cost of the equipment and the cost of the operation, because of the heat required in the evaporation of the excess water and—Second—since dilute sulphuric acid, for instance, vigorously attacks some materials, the entire equipment for this former process of mine must be 30 planned and constructed to resist such attacks, which adds greatly to the cost of the plant and equipment, and also adds to the cost of handling.

In my long study and many experiments along 35 this general line, I have made what I believe to be an important discovery.

If, say, 1 to 10 pounds of water is mixed with a ton of dry sand, the first small fraction of the sand which contacts the water absorbs the entire 40 amount, leaving the balance of the ton of sand completely dry. This is about what anyone would naturally suppose to be the case. My surprising discovery is that if as low as one-half pound of concentrated sulphuric acid is properly 45 mixed with a ton of dry sand, every particle and grain of the sand in the entire ton will be covered by a thin film of concentrated acid; in fact, the result is just as certain, positive and valuable, as if the entire mass were first positively 50 wetted with the dilute acid and the excess water then evaporated by heat, leaving the film of concentrated acid about each particle. If properly handled the mixing of the sand and small amount of acid can be done in a very short time, 55 with some sands in 30 seconds, and the acid will

be evenly distributed through the entire mass of sand.

The explanation of this fact is that concentrated sulphuric acid has very low cohesive power and high adhesive power as compared to 60 water. This can be shown by putting a drop of acid and a drop of water on a plate and then spreading these drops over the plate. The acid drop can be made to cover the entire surface of the plate, while the water drop covers only a 65 small portion of the plate. This test is often performed before students of physics.

I am, therefore, taking advantage of my discovery in regard to sand and other granular materials irrespective of the size of the grain, 70 and, in my present invention, my dry leaching process consists of properly mixing the desired small amount of concentrated sulphuric acid with the dry material and employing heat (which may be applied either before, during, or after the 75 said mixing with the acid) to increase the activity of the acid in attacking the impurities of the material and subsequently removing, by washing or otherwise, the dissolved impurities.

Therefore, I am now, in this invention, going 80 one step further than in my former invention, and am greatly reducing the cost of the necessary equipment and also the operating cost, and still I am accomplishing the desired object of removing those certain impurities from the sand 85 grains, as will appear more in detail hereinafter.

In the operation of this invention I am eliminating the cost of heating the sands or grains to the higher temperatures needed in the former invention, and the evaporation of the diluent. 90

For most sands I now find I need only add the necessary amount of concentrated sulphuric acid to the sand, which has already been dried, agitate or mix it until it is thoroughly mixed with 95 the sand and then allow the mix to stand the necessary time and at the proper temperature, for the acid to act on the impurities.

By using concentrated sulphuric acid, I also, 100 as stated above, do away with the extra cost of acid-proof equipment used in the former process (except in the final washing of the sand) and lower the cost of heating the sand to the much higher temperature formerly used. Sulphuric acid of 60° B. or over does not attack iron or 105 steel can be used.

This new process will effect an operating saving in most sands of between 10 cents to 15 110

cents per ton of sand and will lower the first cost of the plant over 60 per cent.

In the operation of present glass-sand cleaning plants the sand is brought as close as can be to grain size and as much of the dirt, clay, etc. is scrubbed off and washed away. After this cleaning the sand is put through driers, generally either of the Lewiston or rotary type, where the water is evaporated. As the sand comes from the driers it has a temperature of between 130° F. and 250° F. and is practically moisture free. It is then sent to storage bins for shipment.

My process, in its lowest cost form, passes this dry, hot sand, through a suitable type of mixer where the proper amount of concentrated sulphuric acid (the acid must be over 60° B. and should be the commercial "66° B. grade") is added to it. By dry sand is meant a sand so free of moisture that no grains are held together with water and it will run freely as individual grains. The hot sand and acid are then thoroughly mixed. I have found by many tests on sands from all over the country that by properly agitating a mixture of dry sand with as low as one-half pound of concentrated sulphuric acid per ton of sand that the acid spreads over the grains and can be distributed so thoroughly throughout the mass that the iron film on all the sand grains is changed from the oxide to the water-soluble sulphate form and can be washed off. Of course, the heavier the iron film the more acid per ton is needed. As much acid as is found necessary to clean the grains of any particular sand can be added to and mixed with the sand, but very few sands will need over 10 pounds of acid per ton and none will need over 30 pounds per ton of sand to put the iron film into water-soluble form. Dry sand, or ore grains, and concentrated sulphuric acid will thoroughly mix in all proportions from one-half pound of acid per ton of sand up to saturation. Any glass-sand with which I have tried this process will still pour after being properly mixed with the necessary amount of concentrated acid. This is why I call it my dry leaching process.

After mixing the dry sand with the acid it is, in most cases, put in a bin or other receptacle where it is allowed to remain from 15 minutes to 48 hours. The acid acts much more rapidly on some sands than on others. With most sands this time of contact will vary between 4 and 24 hours. Time of contact also varies with the temperature at which the sand is kept in the bin. The usual practice would be to deliver the sand to the mixer at a temperature between 150° F. and 250° F. This sand, after passing through the acid mixer should, for the best results, still have a temperature between 100° F. and 220° F. and should go to the bin within this temperature range. If the sand is too hot, that is over 250° F., a darkening of color may result because of the formation of water-insoluble sulphates. Keeping a temperature of over 212° F. for too long a time may result in this same darkening action, and some sands should not be kept at a temperature of over 200° F. If necessary, the sand can be kept at the correct temperature in the bin by the use of steam pipes or other proper means. If uniformly heated to the proper temperature before going to the bins, no extra heat should be needed. The action of the concentrated acid on the iron film is extremely slow at temperatures ranging below 75° F. As the

temperatures are increased up to the limits above described the needed length of time of contact between the acid and the sand rapidly decreases. As mentioned before, the most efficient range of temperature for the contact step and for the majority of sands ranges between 100° F. and 200° F. Below 100° F. the time of contact is too long for most sands and above 200° F. the chance of forming the dark water-insoluble sulphates is present. However, temperatures to which more finely divided ores and other materials are to be treated depends upon the ore to be treated and the character of impurity to be removed therefrom. But in no case should the temperature of the mixed ore and acid be raised above 560° F.

Concentrated sulphuric acid has the same spreading effect on the dry sand grains even though mixed with the sand at room temperatures. If it is mixed at these temperatures, however, the mixture should then be raised to the above described temperatures and kept at these temperatures for the above mentioned length of time to get the desired results. The addition of heat greatly increases the action of the acid on the impurities and lowers the time of contact required in the bin.

After passing through the bin the acid-covered sand is given a thorough washing in water to rid it of the soluble iron, etc. compounds and remaining free acid. If necessary, a final, very dilute, alkaline wash may be given if the last vestige of free acid must be disposed of. After washing the sand it goes to the drier and is then ready for shipment.

The preliminary crushing, cleaning or desliming of the sand does not concern this process except that as much as possible of the impurities should be removed before adding acid so as to keep down the acid consumption. This cleaning is well done at present and the loose clay and the like, etc. readily removed. Nor does the treatment of the sand after the leach concern this process. Crushers, tables, magnetic machines, and all other equipment may or may not be used for the treatment preliminary to the leach or in the treatment after the leach. This process is only concerned with the removal of harmful impurities such as the iron oxide occurring as a film around the individual sand grains. This film iron is, at present, either not being removed at all or not being removed as cheaply or easily as is done by using the above described method. This process can be added to and made a part of any of the processes of the present sand-cleaning plants. In the case of the smaller grained ores and those that are more finely ground, enough acid should be added thereto so that all of the grains are completely covered therewith. The finer or smaller grains, the greater the total surface area to be covered with the acid. The amount of acid to be added must be sufficient to completely cover all of the surface area of all of the grains and this quantity of acid will naturally increase with the fineness or smallness of the grains to be treated.

The discovery that an extremely small amount of concentrated sulphuric acid can be made, by proper agitation or mixing, to cover with a film of acid a very large number of separate dry grains of granular material appears to be new and no reference has anywhere been found bearing on such action either alone or in connection with the leaching of glass sands.

Having now described my process, what I

- claim as new and desire to protect by Letters Patent, is as follows:
1. The herein described process of purifying dry sand or other granular mineral material comprising adding thereto concentrated sulphuric acid and thoroughly mixing the acid with the material, the amount of acid being sufficient to cover all of the particles of the material with an acid film when said mixing is completed, but not sufficient in quantity to prevent the mixed material and acid from pouring substantially as if dry, employing heat with the sand temperature not over 250° Fahrenheit to energize the action of the acid, storing the mixed acid and material while still heated for a contact period of time and removing the acid and water soluble compounds from the material. 80
  10. The herein described process of purifying dry sand or other granular mineral material comprising adding thereto from one-half pound to thirty pounds of concentrated sulphuric acid per ton of material, thoroughly mixing the acid with the material, storing the material for a contact period of time and subsequently removing the acid and water soluble compounds from the material. 85
  15. The herein described process of purifying dry sand comprising adding thereto concentrated sulphuric acid and thoroughly mixing the acid with the material, the amount of acid added being sufficient to cover all the particles of the material with an acid film when said mixing is completed, but not sufficient in quantity to prevent the mixed material and acid from pouring substantially as if dry, and employing heat with a sand temperature not over 250° Fahrenheit to energize the action of the acid, and subsequently remove from the sand the acid and water soluble compounds. 90
  20. The herein described process of purifying dry sand or other granular mineral material comprising adding thereto between one-half pound and thirty pounds of concentrated sulphuric acid per ton and thoroughly mixing the sand and the acid, and subsequently removing the acid and water soluble compounds from the material. 95
  25. The herein described process of purifying dry sand comprising adding thereto between one-half pound and thirty pounds of concentrated sulphuric acid per ton and thoroughly mixing the acid with the material, and employing heat until the material has a temperature of 250° Fahrenheit or less to energize the action of the acid, and subsequently removing the acid and water soluble compounds from the material. 100
  30. The herein described process of purifying dry sand or other granular mineral material comprising adding thereto between one-half pound and thirty pounds of concentrated sulphuric acid per ton and thoroughly mixing the acid with the material, the amount of acid added being sufficient to cover all of the particles of the material with an acid film when the mixing is completed, but not sufficient in quantity to prevent the mixed material and acid from pouring substantially as if dry, and subsequently removing the acid and water soluble compounds from the material. 105
  35. The herein described process of purifying dry sand or other granular mineral material comprising adding thereto concentrated sulphuric acid and thoroughly mixing the acid with the material, the amount of acid added being sufficient to form an acid film over all the particles of the material but not being sufficient in quantity to prevent the completely mixed material and acid from pouring substantially as if dry, storing the mixed acid and material while still heated for a determined period of time and washing the acid and water soluble compounds from the material and drying the material. 110
  40. The herein described process of purifying dry sand or other granular mineral material comprising adding thereto concentrated sulphuric acid and thoroughly mixing the acid with the material, the amount of acid added being sufficient to cover all the particles of the material with an acid film when the said mixing is completed, but not sufficient in quantity to prevent the mixed material and acid from pouring substantially as if dry, storing the mixed acid and material for a contact period and subsequently removing the acid and water soluble compounds from the material. 115
  45. The herein described process of purifying dry sand or other granular mineral material comprising adding to the material when at a temperature not above 250° Fahrenheit concentrated sulphuric acid, and thoroughly mixing the acid and the material, the amount of acid added being sufficient to cover all of the particles of the material with an acid film when the mixing is completed, but not sufficient in quantity to prevent the mixed material and acid from pouring substantially as if dry, and subsequently removing the acid and water soluble compounds from the material. 120
  50. The herein described process of purifying dry sand or other granular mineral material comprising adding thereto concentrated sulphuric acid and thoroughly mixing the acid with the material, the amount of acid added being sufficient to cover all particles of the material with an acid film when the said mixing is completed, but not sufficient in quantity to prevent the mixed material and acid from pouring substantially as if dry, storing the mixed acid and material for a contact period and subsequently removing the acid and water soluble compounds from the material. 125
  55. The herein described process of purifying dry sand or other granular mineral material comprising adding thereto concentrated sulphuric acid and thoroughly mixing the acid with the material, the amount of acid added being sufficient to cover all the particles of the material with an acid film when the said mixing is completed, but not sufficient in quantity to prevent the mixed material and acid from pouring substantially as if dry, storing the mixed acid and material for a contact period and subsequently removing the acid and water soluble compounds from the material. 130
  60. The herein described process of purifying dry sand or other granular mineral material comprising adding thereto concentrated sulphuric acid and thoroughly mixing the acid with the material, the amount of acid added being sufficient to cover all particles of the material with an acid film when the said mixing is completed, but not sufficient in quantity to prevent the mixed material and acid from pouring substantially as if dry, storing the mixed acid and material for a contact period and subsequently removing the acid and water soluble compounds from the material. 135
  65. The herein described process of purifying dry sand or other granular mineral material comprising adding thereto concentrated sulphuric acid and thoroughly mixing the acid with the material, the amount of acid added being sufficient to cover all the particles of the material with an acid film when the said mixing is completed, but not sufficient in quantity to prevent the mixed material and acid from pouring substantially as if dry, storing the mixed acid and material for a contact period and subsequently removing the acid and water soluble compounds from the material. 140
  70. The herein described process of purifying dry sand comprising adding thereto concentrated sulphuric acid and thoroughly mixing the acid with the material, the amount of acid added being sufficient to cover all the particles of the material with an acid film when the said mixing is completed, but not sufficient in quantity to prevent the mixed material and acid from pouring substantially as if dry, storing the mixed acid and material for a contact period and subsequently removing the acid and water soluble compounds from the material. 145
  75. The herein described process of purifying dry sand comprising adding thereto concentrated sulphuric acid and thoroughly mixing the acid with the material, the amount of acid added being sufficient to cover all the particles of the material with an acid film when the said mixing is completed, but not sufficient in quantity to prevent the mixed material and acid from pouring substantially as if dry, storing the mixed acid and material for a contact period and subsequently removing the acid and water soluble compounds from the material. 150

stantially as if dry and subsequently removing the acid and water soluble compounds from the material.

14. The herein described process of purifying dry sand and other granular material comprising adding thereto concentrated sulphuric acid and thoroughly mixing the acid with the material, the amount of acid being sufficient to cover all the particles of the material with an acid

film when the said mixing is completed, but not sufficient in quantity to prevent the mixed material and acid from pouring substantially as if dry, heating the mixture of material and acid to hasten the chemical action of the acid and subsequently removing the acid and water soluble compounds from the ore.

THEODORE EARLE.

80

85

10

15

90

20

95

25

100

30

105

35

110

40

115

45

120

50

125

55

130

60

135

65

140

70

145

75

150